

Patented June 7, 1927.

1,631,867

# UNITED STATES PATENT OFFICE.

ELIE S. HUMBOLDT, OF OAKLAND, CALIFORNIA, ASSIGNOR TO THE PACIFIC LUMBER COMPANY, OF SAN FRANCISCO, CALIFORNIA, A CORPORATION OF MAINE.

## WOODEN BATTERY SEPARATOR.

No Drawing.

Application filed August 28, 1924. Serial No. 734,815.

This invention relates to the chemical treatment of wood to adapt it for use as storage battery separators, as well as to the products of the treatment including a pre-treated wooden blank adapted for simple shaping to form the finished separator ready for use in the battery.

The objects of the treatment are:—

1st, to remove from the wood as much as possible the deleterious constituents of the ligno-cellulose which may otherwise become hydrolyzed or oxidized by the battery electrolyte during service to form acetic acid and other compounds capable of injuring the battery plates;

2nd, to increase the natural porosity of the wood to allow easier passage of the electrolyte and decrease the internal resistance of the battery.

3rd, to toughen the wood against breakage of the very thin slabs in cutting and finishing the separators therefrom, and from mechanical injury in the battery through pressure and wear of the plates; and all of these in an article adapted for commercial production at the mill point for shipment already treated to the battery separator manufacturer,—something not practicable heretofore on account of wood treated in the ordinary way having a tendency to split if subject to mechanical handling.

The above objects are best secured by my process treating the wood while green, preferably at the mill where it is produced, for I have found that not only is the extraction quicker and more even, but results in an entirely different product, so very much more pliable and tougher, both before and after drying, that it becomes perfectly feasible as a commercial undertaking to manufacture and chemically pre-treat the separator blanks or slabs at the mill and ship them either moist or dry to the battery separator maker for subsequent grooving and finishing to exact dimensions to produce the final separator ready for use in the battery.

This gain in toughness and pliability through treatment of the green wood is a very important feature and probably due to avoidance of any change, hardening, or oxidation of the extractive matter or associated tissue ordinarily produced in drying, for once the wood is dried and then treated there is a marked lowering of its

pliability and toughness which greatly increases liability of breakage and splitting, and which has prevented the commercial quantity preparation of battery separator blanks or slabs at the mill, and the wood has always been reduced to exact size, and surface grooved, by the battery maker, and then variously chemically treated after all mechanical work was done.

My process of treatment is as follows:—

The green wood, is first cut into thin slabs of a thickness corresponding to that of the unfinished separator, generally about one sixteenth of an inch, and of a superficial area a trifle larger than the required separator, or in multiples thereof.

The slabs are then leached in water, either hot or cold, as may best suit the species of the wood being used, to extract the soluble extractive matter, after which the slabs are treated in a hot solution of either an alkali sulphite or of an alkali bisulphite; the sodium salts are generally to be preferred because they are cheap, effective, and do not leave insoluble compounds in the fiber of the wood.

A solution of the salt of from 5 to 12% applied at or near the boiling point for a duration of from 5 to 10 hours will generally yield satisfactory results; however, the best concentration and the time of treatment will vary considerably with the kind of wood being treated, and also depend on its age and lignification, therefore I do not wish to limit myself to any definite concentration or duration of treatment. A few experiments with a particular kind of wood will easily determine the best way of applying my treatment.

When the reaction has been carried to completion, the wooden strips or slabs are immediately washed, preferably in warm water until they are free from both the reagent as well as the reaction products. After washing the slabs may either be partially dried for shaping and finishing, or dried completely for shipping or storing, taking care to preserve the flatness of the slabs during the drying process.

The washing can generally be shortened by first rinsing the slabs thoroughly and then soaking them for a short time in warm water slightly acidulated (about 1%) with sulphuric acid to destroy the last trace of

1. sulphite held by the wood fiber. The resulting sodium sulphate being soluble easily passes out in the washing.

It must be observed that the use of neutral 5 sulphite is more suitable for the treatment of young and soft woods; while the bisulphite, being more energetic, is to be preferred for the older and harder woods, but the use of bisulphite is more liable to yield 10 products which dry hard and brittle unless the action is stopped in time and the final washing done thoroughly.

The finished slab is characterized by its 15 suppleness and its porosity, as the lignocellulose of the hard or winter growth appears to be attacked more deeply than the summer growth, with the result that the wood after treatment has a more even structure than the original material, and also 20 shows a considerable gain in toughness, with less liability of splitting in the subsequent grooving and finishing to the exact separator size.

I claim:-

- 25 1. The process of treating wood for battery separators which comprises reducing the wood while green to substantially the thickness of the desired separators, soaking the green slabs in an aqueous solution of a sulfite or bisulfite at temperatures ranging from 15 C. to the boiling point, and washing out the excess of reagent.
- 30 2. The process of treating wood for battery separators which comprises reducing the wood while green to substantially the thickness of the desired separators, soaking the green slabs in an aqueous solution of a sulfite or bisulfite at temperatures ranging from 15 C. to the boiling point, washing out the excess of the reagent and thereafter 35 drying the wood.
- 40 3. The process of treating wood for battery separators which comprises reducing the wood while green to substantially the thickness of the desired separators, soaking the green slabs in an aqueous solution of a 45

sulfite or bisulfite, treating with acidulated water, and washing.

4. The process of treating wood for battery separators which comprises reducing the wood while green to substantially the thickness of the desired separators, soaking the green slabs in an aqueous solution of a sulfite or bisulfite, treating them with acidulated water, washing, and drying. 55

5. The process of treating wood for battery separators which comprises reducing the wood while green to slab form suitable for cutting therefrom of the desired separators, of chemically treating the slabs while 60 green to remove the deleterious lignone content to adapt the slabs for battery use, and of drying the treated slabs for subsequent mechanical reduction to exact form for use in the battery. 65

6. The process of treating wood for battery separators which comprises reducing the wood while green to slab form suitable for cutting therefrom of the desired separators, of chemically treating the slabs while 70 green to remove the deleterious lignone content to adapt the slabs for battery use, drying the slabs, and thereafter reducing the slabs mechanically to exact size and form for battery use. 75

7. An article of manufacture comprising wooden slabs for battery separators chemically treated while green to remove the deleterious lignone content, and adapted to further mechanical reduction to exact size 80 for the separators.

8. An article of manufacture comprising wooden slabs for battery separators chemically treated while green to remove the deleterious lignone content, and adapted for 85 further mechanical reduction to exact size for the separators without further chemical treatment.

9. An article as specified in claim 7 in which the slabs are each of a superficial area 90 larger than the required finished separator.

ELIE S. HUMBOLDT.